

## UNITED STATES PATENT OFFICE

2,413,718

## LUBRICANT

Bert H. Lincoln, Ponca City, Okla., and Gordon D. Byrkit, Niagara Falls, N. Y., assignors to Continental Oil Company, Ponca City, Okla., a corporation of Delaware

No Drawing. Application November 9, 1942.  
Serial No. 465,084

9 Claims. (Cl. 252—49.7)

1

This invention relates to addition agents and lubricating compositions containing the same and is a continuation-in-part of our copending application, Serial No. 330,950, filed April 22, 1940.

Present-day mechanical devices require lubricating oils of high film strength and of high oiliness characteristics. It has been found that the present-day hydrocarbon lubricants of the very highest quality are deficient in these two very important characteristics. These two properties are of vital importance under conditions of thin film lubrication where the lubricant has been squeezed from between the friction surfaces due to high pressures, slow speeds, and other causes. It is readily seen that the viscosity or the body of the lubricant plays no part in this type of lubrication and that the remaining film of oil should tend to keep the coefficient of friction as low as possible and must have a very high film strength and be of high oiliness value to prevent rupture of the film of the lubricant, which would cause seizure.

Mechanical devices are being designed for higher pressure operation, and the film strength of the best quality straight hydrocarbon lubricants has been found to be too low and not sufficient; therefore an invention which provides the means of improving the film strength of these lubricants is of great importance to the art of lubricant manufacture and to the designer and fabricator of mechanical devices.

Substantially all machines operate in part or at times totally under conditions of boundary or thin film lubrication, under which conditions the oiliness or unctuousness of the lubricant is the first and primary requisite of efficient operation. Those skilled in the art of lubricant manufacture or machine manufacture will readily appreciate the value of an invention that will improve the oiliness of these otherwise high quality lubricants. Under some circumstances, a very small amount of an addition agent will stabilize a hydrocarbon oil against formation of corrosive oxidation compounds or sludge-forming compounds, and as little as 0.001% is often sufficient.

In starting idle mechanical equipment which is lubricated from a sump by pumping or circulating the lubricant, there is always a short period of time during which the rubbing surfaces must operate under conditions of dry friction if ordinary hydrocarbon lubricants are used. With dry friction, the wear on friction surfaces is extreme; and during cold weather when the lubricant is sluggish or during periods when the lubricating system is not functioning properly for one reason or another, rubbing surfaces may not only suffer considerable wear but may be damaged to the point where they must be replaced. The product of our invention has the very important property of reacting with the metal surfaces, pen-

2

trating or adsorbing on the metal, and leaving a film of lubricant with high oiliness character which remains on the metal surface irrespective of the length of time the machine is idle.

This high oiliness film is very even and results in smooth operation which may be easily discerned by the experienced operator and lubricating engineer.

When the hydrocarbon lubricants are diluted with unburned fuel or with other light hydrocarbons, the small degree of oiliness of the original hydrocarbon lubricant is greatly decreased. We have found that the addition of the product of our invention to hydrocarbon lubricants more than compensates for the loss in oiliness and load-carrying ability by dilution.

One object of our invention is to provide a lubricating composition having improved film strength and extreme pressure characteristics.

Other and further objects of our invention will appear from the following description.

We have found that certain compounds are adsorbed or absorbed by metals forming a plurality of layers or films on the surface of the metal, which films are very tenacious (they have a high film strength) and have the property of reducing the coefficient of friction to a greater extent than any known lubricant. The compounds which most readily are adsorbed by metals are ones consisting of polar molecules, that is, molecules of unsymmetrical electrical character which contain an atom or group of atoms exhibiting a secondary or residual valence. These polar compounds tend to produce regimentation of the molecules of hydrocarbon oil when added thereto. If a metal is immersed in a strongly polar compound, a regimentation or cybotaxis of the molecules will take place in the adsorbed film, the molecules being oriented with respect to the surface of the metal by which they are adsorbed. The films of polar compounds, adsorbed by a metal, can be plainly seen and the orientation of the polar molecules on the metal surface ascertained by X-ray diffraction methods, in which a monochromatic X-ray beam is passed through the adsorbed films at an angle. The series of films acts as a diffraction grating, and a diffracted beam will be reflected from the planes of the films and can be recorded photographically. The X-ray photographs will clearly show the orientation of the molecules by characteristic pictures.

X-ray investigation has shown that strongly polar molecules form adsorbed films of unusual thickness and regularity of arrangement. Thicknesses of films of 9,000 Angstrom units have been obtained, which are of enormous magnitude when compared with molecular dimensions.

Broadly stated, our invention comprises the making available for use as addition agents in lubricating compositions of halogen bearing or-

gano-boron esters of the type which contain the  $>B-OR$  group (in which R is an organic radicle) and improved lubricating compositions containing minor amounts of such addition agents.

The use of organo-boron compounds broadly in lubricating compositions is not new. Their principal use in lubricating compositions is disclosed in Patent No. 2,234,581, wherein acidic organo-boron compounds are disclosed for the purpose of preventing oxidation of lubricants, especially when the same are subjected to high temperatures and gases which tend to promote oxidation. That patent, as indicated, relates to the use of acidic materials, and the amounts specified for use are in all cases "minute." While organic-substituted boric acids, that is, compounds having the  $>B-OH$  group, are disclosed therein, these are described as being of low solubility and less desirable.

In addition to the disadvantage of low oil-solubility, the acidic organo-boron compounds are corrosive to sensitive bearing metals, such as are commonly used in modern internal combustion engines.

We have found, however, that a much more satisfactory sub-generic class of organo-boron compounds for the foregoing uses are those of the ester type and which are additionally characterized by the presence of combined halogen in the molecule.

The ester type material is preferable for use in that it does not have the objectionable high reactivity above pointed out which is possessed by the acidic material. In the same concentrations as suggested by the prior art for the acidic type material, our ester type material is quite effective from the standpoint of inhibiting oxidation without, however, possessing the undesirable properties of the acidic material. The additional characteristic of our improved addition agent, namely, that it contains halogen, gives rise to further advantages, the most important of which may be enumerated as follows:

The presence of halogen in the molecule renders the compounds much more strongly polar, and accordingly they are attracted to the metallic surfaces with which the lubricant comes in contact and which the lubricant is designed to protect from scuffing and scoring, due to overload and the like. This strongly polar nature of the compounds makes it possible to achieve effects on the metal surfaces, such as the bearings, which are not only impossible by the prior art uses of the acidic materials, but which the prior art deliberately sought to avoid by keeping down to as low as possible the concentrations within which such acidic materials were employed.

The addition agents of our invention are desirably strongly polar for the reason that one of the principal purposes for which they are present in the lubricating compositions of our invention is dependent upon their ability to react in a chemical or physico-chemical fashion with the bearing surfaces being lubricated. This chemical or physico-chemical action by which the addition agents of our invention improves the lubricating compositions containing the same is two-fold, and the effects thereof are likewise two-fold.

In the first place, the strongly polar nature of the addition agents causes the same to be oriented as an adsorbed film on the bearing surfaces sought to be lubricated with the attended advantages, such as higher "oiliness"; less tend-

ency of the lubricant to drain from the bearing surfaces, etc., all as previously explained.

A second and equally important effect of the increased polarity of our improved addition agents is the increased film strength of the lubricant containing the same, attributable to the function of the cooperative effect of the halogen and the  $R>BOR'$  group present in the molecule as a film strength improver.

The presence of halogen in the molecule has an additional advantage in that it renders the compound much less volatile so that it will not be so readily evaporated from the lubricating compositions during use at high temperatures. At this point it may be well to note that for most purposes the addition agents should have a vapor pressure less than atmospheric at a temperature of 140° C. and preferably at 170° C.

When one of the desired effects of the presence of the addition agent is an increase in the film strength of the lubricant, the ester materials of this invention are particularly advantageous because their higher solubility, as compared with the acidic materials of the prior art, makes it

possible to incorporate amounts which are much more effective for that purpose; that is, in amounts higher than .75% or preferably above 1.0%. The upper limit of the concentration of addition agents is determined by factors such as the limit of their solubility; reasons of economy, etc. Our invention, therefore, contemplates that these addition agents may be used in lubricating compositions such as those which comprise a mineral oil base in effective amounts up to the limits of their solubility in the oil, there being generally no reason, however, for including more than about 20%.

The broad class of organo-boron esters contemplated for use by this invention contains two important sub-divisions respectively represented by the following formulas:



in which R and R' are organic radicles and X is a radicle of the class consisting of  $-R''$  and  $-O-R'''$  where R'' and R''' are organic radicles; and



in which  $R^d$  is a divalent organic radicle, and R is an organic radicle.

Other sub-divisions of the broad class of esters contemplated hereby are the following:

$R>BOR'$ , in which R and R' are organic radicles, at least one of which contains four or more carbon atoms. An example of this type is chlorodiethyl boric acid lauryl ester.

$RB(OR')_2$ , in which R and R' are organic radicles, at least one of which contains four or more carbon atoms. An example of this type is chlorophenyl boric acid dilauryl ester.

These two types of organo-boron esters have the general formula  $R_nB(OR')_{3-n}$  where n is an integer less than 3, the valence of boron. They contain at least one carbon-boron bond, and at least one organic radicle is removable by saponification. R and R' are usually hydrocarbon radicles but are not necessarily hydrocarbon radicles, and they may contain besides carbon and hydrogen also other elements including oxygen, sulphur, halogen, phosphorus, or metals. Other examples of our compounds are chlorophenylboric

acid dibutyl ester, chlor diamylboric acid cyclohexyl ester, and the like.

Examples of the organic radicles represented by R, R', R'', R''' and R<sup>d</sup>, referred to throughout all of the foregoing description, are the following: 5

A. Hydrocarbon radicles

1. Alkyl radicles

Amyl (n, iso, sec. and tertiary)

Octyl

Lauryl

Cetyl

Carnaubyl

Ceryl

Montanyl

Mellisyl

Myrcyl

Lacceryl

Psylleryl

10

2. Aryl radicles

Phenyl

Xenyl

Naphthyl (alpha- and beta-)

Anthracyl

Phenanthryl

15

3. Cyclo-alkyl radicles

Cyclopentyl

Cyclohexyl

Cycloheptyl

Cyclohexyl-cyclohexyl

20

4. Alkylated aryl radicles

Radicles formed by the alkylation of aryl radicles, such as those listed above (2), with any of the alkyl radicles, e. g., those listed above (1), or with any of the following:

25

Methyl

Ethyl

Propyl (n- and iso-)

Butyl (n-, iso- and sec-)

Specific examples of alkylated aryl radicles are as follows:

Cresyl

Xylyl

Trimethyl-phenyl

Ethyl-phenyl

Tetra-ethyl-phenyl

t-Amyl-phenyl

Lauryl-phenyl

Cetyl-phenyl

Ceryl-phenyl

Methyl-naphthyl

Iso-propyl-naphthyl

t-Amyl-naphthyl

Lauryl-naphthyl

Cetyl-naphthyl

Iso-propyl-xenyl

t-Amyl-xenyl

Lauryl-xenyl

30

5. Alkylated cyclo-alkyl radicles

Radicles formed by the alkylation of cycloalkyl radicles, such as those listed above (3), with any of the alkyl radicles, such as those listed above.

Specific examples are:

Methyl-cyclohexyl

Dimethyl cyclohexyl

t-Amyl cyclohexyl

Lauryl cyclohexyl

Cetyl cyclohexyl

Menthyl

Fenethyl

Bornyl

40

6. Cyclo-alkylated aryl radicles, e. g.

Cyclohexyl-phenyl

50

Cyclohexyl-xenyl

Cyclohexyl-naphthyl

7. Arylated-alkyl radicles, e. g.

Benzyl

Phenyl-ethyl

Phenyl-amyyl

Phenyl-lauryl

Phenyl-cetyl

Xenyl-methyl

Xenyl-ethyl

Naphthyl-methyl

Naphthyl-ethyl

55

8. Cyclo-alkylated alkyl radicles, e. g.

Naphthetyl

Hexahydrobenzyl

Cyclohexyl-ethyl

Cyclohexyl-amyyl

60

9. Arylated cyclo-alkyl radicles, e. g.

Phenyl-cyclohexyl

Xenyl-cyclohexyl

Naphthyl-cyclohexyl

10. Mixed radicles, e. g.

Methylcyclohexyl-phenyl

Amylcyclohexyl-phenyl

Cyclohexyl-cresyl

Cyclohexyl-lauryl

Cyclohexyl amył-phenyl

Cyclohexyl-benzyl

Xylyl-cyclohexyl

Lauryl-phenyl cyclohexyl

Cetyl-phenyl cyclohexyl

Phenyl-methylcyclohexyl

Phenyl-amylcyclohexyl

Xylyl-methylcyclohexyl

Benzyl-cyclohexyl

Benzyl-methylcyclohexyl

Methylcyclohexyl-amyyl

Methylcyclohexyl-lauryl

65

70

75

A. Hydrocarbon radicles—Continued.

11. Divalent hydrocarbon radicles

Methylene

Ethylene

Ethylidene

Vinylene

Vinylidene

Propylene

Propylidene

Isopropylidene

Propenylidene

Butylene

Butylidene

Isobutylidene

Amylene

Amylidene

Iso-amylidene

Cyclohexylene

Cyclohexylidene

Phenylene

Phenylidene

Benzal

Cinnamal

Styrolene

Naphthylene

Naphthylidene

Naphthal

Tolylene

Xylylene

Biphenylene

Vinyl

Allyl

Propenyl (n, and iso-)

Butenyl (n-, and iso-)

Oleyl

Cyclohexenyl

Styryl

Cinnamyl

12. Unsaturated hydrocarbon radicles

B. Oxygen-containing organic radicles

1. Of the ether type, e. g.

Methoxy-phenyl (anisyl)

Anisal

Ethoxy-phenyl (phenetyl)

Lauroxy-phenyl

Cyclohexoxy-phenyl

Phenoxyl-phenyl

Phenoxyl-naphthyl

Phenoxyl-cyclohexyl

Phenoxyl-ethyl

Phenoxyl-lauryl

Phenoxyl-cetyl

Phenoxyl-ethoxy-ethyl

—C<sub>6</sub>H<sub>4</sub>—O—C<sub>2</sub>H<sub>4</sub>— (derived from di-ethylene glycol)

—C<sub>6</sub>H<sub>4</sub>—O—C<sub>6</sub>H<sub>4</sub>— (derived from diphenyl ether)

Furyl

Fural

2. Of the ketone type, e. g.

Acetyl

Acetyl-phenyl

Acetyl-xenyl

Acetyl-naphthyl

Acetyl-lauryl

Acetyl-cetyl

Acetyl-cyclohexyl

Acetyl-naphthyl

Crotonyl

Phenacyl

Phenacylidene

Lauroyl

Lauroyl-phenyl

Benzoyl

Benzoyl-phenyl

Benzoyl-naphthyl

Benzoyl-cyclohexyl

Benzoyl-naphthene

Benzoyl-lauryl

Benzoyl-cetyl

Stearoyl

Stearoyl-phenyl

Stearoyl-xenyl

Stearoyl-naphthyl

Stearoyl-amyl

Stearoyl-lauryl

Stearoyl-cetyl

Stearoyl-phenoxyphenyl

Stearoyl-cyclohexyl

Stearoyl-naphthene

Herahydrobenzyl

Naphthenoyl

Naphthenoyl-phenyl

Naphthenoyl-xenyl

Naphthenoyl-naphthyl

Naphthenoyl-amyyl

Naphthenoyl-lauryl

Naphthenoyl-cetyl

Naphthenoyl-phenoxyl-phenyl

Naphthenoyl-cyclohexyl

Phenoxylbenzoyl-phenyl

Lauryl-benzoyl

Cetyl-benzoyl

Anisoyl

Cinnamoyl

Naphthoyl

Salicylyl

Toluyl

Xyloyl

Furoyl

—C<sub>6</sub>H<sub>4</sub>—CO—C<sub>6</sub>H<sub>4</sub>— (derived from salicyl-phenol)

Acetonyl

Acetonylidene

Acrylyl

B. Oxygen-containing organic radicles—Continued.  
2. Of the ketone type—Continued.

Adipyl

Benzoylene

Butyryl

Isobutyryl

Carbethoxy

Cresotyl

Desyl

Glutaryl

Glycolyl

Melonyl

Oxalyl

Phthalyl

Succinyl

3. Of the ester type, i. e.

Derived from hydroxy-esters by the removal of the hydroxyl group, as for example, by the removal of the hydroxyl group from the following esters:

a. Esters of hydroxy acids, e. g.

Esters formed by substitution of any of the "R" groups listed above for one or more of the acid hydrogen atoms of the following acids:

Lactic acid

Hydrylic acid

Citric acid

Tartaric acid

Ricinoleic acid

Hydroxy-stearic acid

Hydroxy-chlorstearic acid

Cyclohexanol carboxylic acids

Hydroxybenzoic acids

Salicylic acid

Hydroxy-phthalic acids

Hydroxy phenyl-benzoic acids

Naphthol carboxylic acids

Esters of polyhydroxy alcohols and phenols in which at least one hydroxyl group remains unsubstituted, for example—esters formed by esterifying the following so that at least one hydroxyl group remains in the resulting ester:

Ethylene glycol

Diethylene glycol

Propylene glycols

Butylene glycols

Poly-hydroxy benzenes

Dihydroxy-benzenes

Resorcinol

Catechol

Hydroquinone

Tri-hydroxybenzenes

Pyrogallol

4. Hydroxy radicles

Hydroxy-ethyl

Hydroxy-butyl

Hydroxy-ethyl

Hydroxy-phenyl

Hydroxy-benzyl

Hydroxy-cyclohexyl

Amyl hydroxy-phenyl

Lauryl hydroxy-phenyl

Cetyl hydroxy-phenyl

Di-amyl hydroxy-phenyl

Lauryl hydroxy-benzyl

Amyl hydroxy-cyclohexyl

Phenyl hydroxy-phenyl

Phenyl hydroxy-benzyl

Hydroxyphenyl-phenyl

Hydroxyphenyl-benzyl

Hydroxybenzyl-phenyl

Hydroxybenzyl-phenyl

Hydroxy-benzoyl

Hydroxy-stearoyl

Salicylal

## C. Sulphur-containing organic radicles.

Examples are any of the radicles listed under B in which a sulphur atom has been substituted for one or more oxygen atoms, e. g.,

R—S—R'

S  
||  
R—C—S  
||  
R—C—R', etc.where R is an aliphatic radicle (e. g., methyl, ethyl, butyl, lauryl), a cyclo-aliphatic radicle (e. g., cyclohexyl, methyl-cyclohexyl) or an aromatic radicle (e. g., phenyl, benzyl, tolyl, xenyl, naphthyl), and R' is a divalent organic radicle, e. g., methylene, ethylene, amylene, phenylene,  $-\text{C}_6\text{H}_4-\text{CH}_2-$ ,  $-\text{C}_6\text{H}_4-\text{C}_6\text{H}_4-$ , $\text{CH}_2-$   
 $-\text{C}_6\text{H}_4-$   
hexahydrophenylene,  $-\text{C}_6\text{H}_{10}\text{CH}_2-$ ,  $-\text{C}_6\text{H}_{10}-\text{C}_6\text{H}_{10}-$ , etc.

Specific examples are:

Thiomethoxy-phenyl ( $\text{CH}_3-\text{S}-\text{C}_6\text{H}_4-$ )Thiophenoxy-ethyl ( $\text{C}_6\text{H}_5-\text{S}-\text{C}_2\text{H}_5-$ )Thiocyclohexoxy-phenyl ( $\text{C}_6\text{H}_{11}-\text{S}-\text{C}_6\text{H}_4-$ )

Thio-acetyl

Thio-stearoyl

Thio-naphthenoyl

Thio-benzoyl

Thio-benzoyl-phenyl

Thio-stearoyl-phenyl

Thio-stearoyl-phenyl

Thio-acetyl-phenyl

## C. Sulphur-containing organic radicles—Continued.

Specific examples—Continued.  
Thio-acetyl-benzyl  
Mercapto-phenyl  
Mercapto-benzyl  
Mercapto-ethyl  
Mercapto-butyl  
Mercapto-benzoyl  
Mercapto-stearoyl  
Mercapto-thio-benzoyl  
Mercapto-thio-stearoyl  
Mercapto-thio-stearoyl-phenyl  
Mercapto-thio-benzoyl-phenyl  
Lauryl mercapto-phenyl  
Lauryl mercapto-benzyl  
Thienyl  
Thiazyl

It is to be understood that the foregoing organic radicles may have one or more atoms of halogen, and more specifically of chlorine, substituted for one or more hydrogen atoms in the preparation of the halogen bearing esters which comprise the addition agents of this invention.

Esters of the type RR'BOR'', or R<sub>2</sub>BOR'' may be made by replacing one ester group of a triester by reacting the ester with only enough Grignard reagent of the formula RMgBr to carry the reaction just one step. The second step may then be carried out with the same Grignard reagent, or a different one, R'MgBr, depending on whether R and R' are to be the same or different.The esters of type RB(OR')<sub>2</sub> may be prepared as follows:

The triester is reacted with RMgBr →

R and R' may be any organic radicles, for example ethyl and  $\text{CH}_2\text{CH}_2\text{CH}_2\text{CH}_2\text{Cl}$  respectively.

40 The above type reaction makes use of the Grignard reagent and reaction. The above reaction would give a product in which the R's are the same.

45 It is possible to use phenyl, chlorphenyl, naphyl, aliphatic, aliphatic substituted aromatic, and aromatic substituted aliphatic radicles to form the triester. It is preferable to have the chlorine in the radicles prior to the reaction.

By varying the alcohol and the Grignard reagent it would be possible to obtain a great variety of esters.

An aromatic radicle may be placed in the ester linkage in the following way:



9

This triester can be reacted with any Grignard reagent to obtain the ester containing a carbon to boron linkage.

Specific examples of the organo-boron esters of this invention are:



10



20 where M is a divalent metal, e. g., the alkaline earth metals.

25 It is sometimes advantageous to combine more than one of these compounds in a blend to obtain particular properties. We accomplish this by mixing two or more of these compounds together and blending the mixture with hydrocarbon oil, or by blending one in the hydrocarbon oil, blending the second into this mixture, and so on until the composition is complete.

30 We have found that the organic boron compounds above set forth may be more effective in some compositions if a comparatively small amount of halogen-free, oxygen-containing carbon compound is included in the composition. The oxygen-containing carbon compound may be 35 of aliphatic, aromatic, or hetero-cyclic nature and may be blended with the organic boron compound in amounts ranging from 5 to 50 per cent.

35 It will be understood that certain features and sub-combinations are of utility and may be employed without reference to other features and sub-combinations. This is contemplated by and is within the scope of our claims. It is further obvious that various changes may be made in details within the scope of our claims without departing from the spirit of our invention. It is, therefore, to be understood that our invention is not to be limited to the specific details shown and described.

40 Other modes of applying the principle of the invention may be employed, change being made as regards the details described, provided the features stated in any of the following claims or the equivalent of such be employed.

45 We therefore particularly point out and distinctly claim as our invention:

50 1. A lubricant comprising in combination a major proportion of a hydrocarbon oil and from .001% to about 20% of an oil-soluble halogen-bearing ester containing at least one carbon-boron bond.

55 2. A lubricant comprising in combination a major proportion of a hydrocarbon oil and from .001% to about 20% of an oil-soluble halogen-bearing organo-boron ester containing at least one carbon-boron bond and having the formula:



65 in which R and R' are organic radicles, X is a radicle of the class consisting of —R'' and —O—R''' where R'' and R''' are organic radicles.

70 3. A lubricant comprising in combination a

## 11

major proportion of a hydrocarbon oil and from .001% to about 20% of an oil-soluble halogen-bearing organo-boron ester containing at least one carbon-boron bond and having the formula:



in which  $R^d$  is a divalent organic radicle and  $R$  is an organic radicle.

4. A lubricant comprising in combination a major proportion of a hydrocarbon oil and from .001% to about 20% of a halogen-bearing organo-boron ester containing at least one carbon-boron bond and having the formula  $R_nB(OR')_{3-n}$  in which  $R$  and  $R'$  represent organic radicles and  $n$  is an integer less than 3.

5. A lubricant comprising in combination a major proportion of a hydrocarbon oil and from .001% to about 20% of a halogen-bearing organo-boron ester containing at least one carbon-boron bond and having the formula  $RB(OR')_2$  in which  $R$  and  $R'$  are organic radicles.

6. A lubricant comprising in combination a major proportion of a hydrocarbon oil and from

## 12

.001% to about 20% of a halogen-bearing organo-boron ester containing at least one carbon-boron bond and having the formula  $R_2B.OR'$  in which  $R$  and  $R'$  are organic radicles.

5. A lubricant comprising in combination a major proportion of a hydrocarbon oil and a minor proportion of an oil-soluble halogen-bearing organo-boron ester containing at least one carbon-boron bond and containing an alkaline-earth metal in the molecule.

10 8. A lubricant comprising in combination a major proportion of lubricating oil and from .001% to about 20% of chlorphenylboric acid dibutyl ester containing at least one carbon-boron bond.

15 9. An extreme pressure lubricating composition comprising a major proportion of a lubricating oil and from .75% to about 20% of a halogen-bearing organo-boron ester containing at least one carbon-boron bond.

BERT H. LINCOLN.  
GORDON D. BYRKIT.